

## UNITED STATES PATENT OFFICE

1,998,576

NOVEL ARTIFICIAL SILK EFFECTS AND  
PROCESS OF PRODUCING SAME

Georges Heberlein, Wattwil, Switzerland, assignor to Heberlein Patent Corporation, New York, N. Y., a corporation of New York

No Drawing. Application January 13, 1927, Serial No. 161,022. In Germany January 15, 1926

16 Claims. (Cl. 8—20)

My invention relates to novel artificial silk effects and process of producing same. The object of the invention is to provide artificial silk goods having their physical characteristics 5 changed or altered in one or more respects, such as a change in the characteristic appearance and/or hand (touch). I use the term "artificial silk" in this specification and in the appended claims as designating the various forms of regenerated cellulose such for example as artificial silks known as viscose, cuprammonium and nitrocellulose silks, the latter being exemplified, for example, by those known in commerce as Chardonnet & Tubize; and as excluding acetate 10 silk.

According to the invention, for example, artificial silk (regenerated cellulose but not acetate silk) may be so treated that the characteristic excessive lustre of artificial silk fabrics will partially or wholly disappear and the fabric will assume a lustreless, transparent effect, and become stiffer to the touch. As will be more fully explained according to this invention, a variety 20 of novel effects in artificial silk may be obtained, and some of these effects are especially valuable in the production of pattern effects on fabrics made entirely or partly of artificial silk fibres.

The process is applicable to artificial silk 30 goods whether in the form of yarn (threads) or fabric (in the piece), and whether the thread or the fabric is made entirely or only partly of artificial silk.

The ennobling of cotton fibres by means of 35 swelling agents is known. It is possible thereby to impart upon the fibre a lustrous appearance by mercerization and to produce thereon transparent and/or wool like effects by means of concentrated acids, according to conditions.

When cellulosic material such for example as 40 natural cotton fibres or regenerated cellulose is acted upon by a swelling agent the swelling action or the structural change brought about in the fibre is dependent upon certain factors, i. e., concentration of the swelling agent and time 45 of treatment, and with most swelling agents upon the temperature of the agent. This is now well known with respect to cotton fibres. If the concentration is too low the swelling action will not take place in a given fibre, no matter how prolonged the time of treatment may be, and also if the concentration is sufficient to produce the desired effect on a particular fibre when applied for a sufficient time; if not applied for a suffi- 50 cient time there will be no or substantially no

swelling action. Likewise utilizing a suitable concentration for the desired effect on a particular fibre, if the time of treatment is too long the particular fibre may be destroyed or spoiled. As is also now understood, variations 5 in temperature of most of the swelling agents permit of variations in one or both of the other factors—concentration and time of treatment.

The degree of capability of a swelling treatment to attack or alter cellulose fibres, I will 10 designate for brevity and convenience herein as the "severity" of treatment. For example, if sulphuric acid of say 54° Bé. is allowed to act at a given temperature upon a previously mercerized cotton fabric for say 5 seconds, and a certain 15 swelling action is obtained, the "severity" of such treatment will be less than one utilizing the sulphuric acid at a concentration of 58° Bé. and at the same temperature for the same duration; the "severity" of treatment being measured 20 by the extent to which the fibres are attacked by the treatment.

Now I have discovered that the character of 25 swelling action brought about in the fibres (regenerated cellulose) is also determined by the above factors,—concentration, time, and temperature of the swelling agent, and that swelling treatments which are of suitable "severity" for producing desirable swelling actions on natural 30 cotton fibre or fabric, are too severe for the treatment of artificial silk (regenerated cellulose) and will destroy the same, but that such 35 artificial silk can be successfully treated with swelling agents to produce various desirable permanent effects provided the "severity" of treatment with the swelling agent is less than that capable of producing any or any substantial swelling action on the ordinary or natural cotton fibre or fabric.

While it is impossible to specify the exact factors, i. e., concentration, time of treatment and temperature, for every desired effect on the artificial silk, due to the numerous variety of effects that may be desired and the various conditions under which the artificial silk is to be 45 treated, nevertheless, in view of the foregoing general rule taken in connection with the specific examples of treatments and other information hereinafter given, those skilled in the art will be able to determine the swelling agent and 50 the desired factors of time, concentration and temperature for the treatment of any particular artificial silk (regenerated cellulose) for a particular finish or effect.

According to this invention valuable changes 55

on artificial silk can be produced by means of swelling agents, whereby novel characteristics, not known before on artificial fibres, are obtained. Such swelling agents are: alkali—hydroxide of concentrations as generally used for mercerization, i. e. of a density of above 10° Bé., sulfuric acid of a density of above 42° Bé., phosphoric acid of a density of above 50° Bé., muriatic acid of a density of above 20° Bé., nitric acid of a density of above 35° Bé. as well as mixtures of the above-mentioned acids; concentrated salt solutions, i. e. chloride of zinc solution of a density of above 50° Bé., calciumrhodanide solution of a density of above 25° Bé., copperoxideammonia solution with at least 0.3% copper content; but from the commercial standpoint the most desirable of these swelling agents for treating artificial silk are, caustic soda, sulphuric acid, nitric acid and the nitration acid mixtures. Additional substances as proposed for lessening the speed of the reaction can also be added to these agents; among which substances are included one or more univalent and/or multivalent alcohols heterocyclic bases, formaldehyde and ammonia salts.

In treating artificial silk during longer or shorter periods according to the kind and concentration of the swelling agents, and in conformity with prevailing operating temperatures, the same loses a part of its excessive lustre and, quite in contrast to the reflection of light which is otherwise predominant above everything else, it becomes transparent or translucent; and gradually an effect develops similar to the known transparent or glass like batiste effects on cotton. If desired, by means of variations in the concentration; temperature and time of action any intermediate grade between the high lustrous character of the original material and the dull, glass-like transparent, stiff, final product can be obtained.

By such treatments, the artificial silk obtains new characteristics unknown before. It has been discovered that just at the beginning of the action, when no extensive swelling has taken place, and hence almost the full lustre is still present, especially in fabrics of artificial silk, an unexpected equalization of the fabric structure takes place, thus causing the unpleasant stripes, which very often appear in artificial silk, to disappear. Also if the swelling of the artificial silk is not continued beyond the permissible measure, then a remarkable increase of the tensile strength is observable; this is due to surface adhesion of the single fibres or filaments.

Each of the mentioned reagents alter artificial silk in a similar manner as above described; that is, they all act to increase the stiffness and translucency of the artificial silk fabric, and many of them to reduce or entirely eliminate the excessive lustre. But in the use of nitrating acid (a composition containing varying proportions of sulphuric and nitric acid with varying aqueous content) widely varying and different effects are produced depending upon the ratio of the nitric acid to the sulphuric acid and upon the aqueous content of the mixture.

For example, if the nitrating acid has an aqueous content below 20%, then quite different effects are produced upon the artificial silk depending upon whether the nitric acid content or the sulphuric acid content predominates. For example if more nitric than sulphuric acid is present the result will be an entirely lustreless non-translucent product; whereas if the sul-

phuric acid predominates the result will be a voluminous soft rich lustre effect of crepe-like character more nearly like natural silk. But if the nitrating acid contains 20% or more water then regardless of whether the nitric or sulphuric acid predominates, the result is similar to that with the use of the other reagents, i. e., a diminishing of the high lustre and increased stiffness and transparency.

It will thus be seen that one may produce various effects by the use of different mixtures of sulphuric and nitric acids. Such nitrated products may be subsequently treated with known denitrating means to rid them of their ready inflammability.

The manipulation of artificial silk is mostly carried out at normal temperature, but also low temperatures can advantageously be employed, whereas in the use of salt solutions often the warming of agents, some to above the boiling point of water, is necessary. The acting period can be from a few seconds to several minutes, according to the desired effect, in individual cases up to one hour. The fibre material is held loose or under tension in the swelling agents depending upon the effect desired.

The process is applicable to all kinds of artificial silks of regenerated cellulose, but not to acetate silk. They may be treated loose, spun or woven or as a formation of any kind, alone or also mixed with other fibres. Also those fibres, designated as staple fibre, and products obtained by spinning of short single fibres, are susceptible to this ennoblement.

#### Examples

1. Bleached artificial silk fabrics are passed through caustic alkali of 20° Bé. for a period of 4 seconds at normal temperature and slight tension, washed out, soured with diluted sulphuric acid, thoroughly washed and dried. The fabric becomes stiff, translucent, and still exhibits a faint lustre.

2. De-sized artificial silk fabric is passed through a bath cooled to minus 10° C. of sulphuric acid of 49° Bé. during 5 seconds, washed completely free from acid and dried. The fabric becomes somewhat stiffer, still shows a high lustre though slightly reduced, has become slightly translucent and appears much more uniform in structure; that is to say, the above-mentioned equalization of the fabric structure is apparent.

3. Immerse artificial silk fabrics at normal temperature during 5 minutes into nitric acid of 40° Bé. wash out well and dry. The fabric shows a high lustrous, translucent effect with considerable stiffness of the fabric.

4. Artificial silk yarn is impregnated for a period of 10 minutes in a nitrating acid mixture, consisting of 4 parts sulphuric acid and one part nitric acid with an aqueous content of 7%, then washed and dried. The fibre becomes voluminous, soft, and acquires the rich lustre of real silk.

5. Artificial silk fabrics are passed through a chloride of zinc solution of 67° Bé. at 40° C. during a period of 10 seconds, washed out and dried. The fabric has become translucent and loses its lustre. Those skilled in the art will observe from a consideration of the foregoing five specific examples of treatments according to the present invention, that in each case the factors of concentration, temperature and duration of treatment are so chosen that the "severity" of treatment is insufficient to produce any or any substantial

swelling action on natural cotton fibres. Taking for illustration the treatment of Example 1, while the caustic alkali is of ordinary mercerizing strength yet the period of treatment is but 5 four seconds at normal temperature as contrasted with the duration of treatment of from 8 to 12 seconds for mercerizing.

If the above named swelling agents are allowed to act upon localized portions of fabrics, which 10 contain artificial silk, these portions are affected, producing contrast between treated and untreated portions, which is enhanced by dyeing due to different affinities for certain dyes.

This fact can be of use for producing patterned 15 effects. The local action of the swelling means can be done by applying to the fabric directly, by printing, blowing or painting, reserves with or without thickening means, and the fibre material is subsequently immersed in the swelling 20 means. Dyestuffs can be added to the reserves, by which a local color effect can be produced together with the reserve.

The process can be used on all kinds of 25 material made of artificial fibres consisting of regenerated cellulose. Materials made of artificial silk mixed with natural vegetable and animal fibres can be thereby treated.

In treating mixed materials it has been discovered, that it is advantageous for producing 30 soft effects if the natural fibres, such for example as cotton, are worked up in the grey condition and are only cleaned or bleached after the local action of the swelling agents thereupon. By this means the end is attained that the natural fibres, 35 in consequence of their natural incrustations, are not so quickly affected by the swelling agents, i. e., are not affected during the time required for altering the regenerated fibres, and therefore retain their original construction. If artificial 40 fibres and both raw and already disintegrated natural fibres are employed side by side in mixed fibres, the variety of the effects is further increased, a result that makes itself evident particularly in subsequent dyeing.

45 Where in the appended claims I use the term "artificial silk" I wish to be understood as including regenerated cellulose in the form of fibres, threads or fabric, and whether or not, in the case of threads, they also contain cotton or other fibres; and whether or not, in the case of fabric, it also contains cotton or other threads. Also I wish to be understood by the term "artificial silk fabric" as used in the claims, to include fabrics made either wholly of regenerated 50 cellulose fibres or of mixtures of same with other fibres.

Such features of my invention as to product 60 and process, not herein claimed, will be the subject of one or more copending divisional applications.

Having thus described my invention, what I claim as new and desire to secure by Letters Patent, is:

65 1. Process for producing a novel character of artificial silk, which comprises subjecting the artificial silk to the action of a swelling agent which will chemically structurally change the same to effect a change in at least one of its natural physical characteristics:—lustre, stiffness, 70 translucency, said treatment being of sufficient "severity" to effect said change but less than that capable of producing any substantial swelling action on natural cotton fibres.

75 2. Process for producing a novel character of

artificial silk, which comprises subjecting the artificial silk to the action of a swelling agent which will modify its characteristic lustre and increase its stiffness, said treatment being of sufficient "severity" to effect said change but less than that capable of producing any substantial swelling action on natural cotton fibres.

5

3. Process for producing a novel character of artificial silk, which comprises subjecting the artificial silk to the action of a swelling agent 10 which will modify its characteristic lustre and render it stiffer more translucent, said treatment being of sufficient "severity" to effect said change but less than that capable of producing any substantial swelling action on natural cot- 15 ton fibres.

4. Process for eliminating the characteristic high lustre of artificial silk, which comprises subjecting the same to the action of alkali hydroxide of lustre-eliminating strength, said treatment 20 being of sufficient "severity" to effect said change but less than that capable of producing any substantial swelling action on natural cotton fibres.

5. Process for producing pattern effects on 25 artificial silk fabric, which comprises subjecting localized portions of the fabric according to pattern to the action of a swelling agent which will chemically structurally modify at least one of the characteristics:—lustre, stiffness, translucency, so as to produce said pattern effect by contrast 30 with the untreated portions, said treatment being of sufficient "severity" to effect said change but less than that capable of producing any substantial swelling action on natural cotton fibres.

6. Process for producing pattern effects on 35 artificial silk fabric, which comprises subjecting localized portions of the fabric according to pattern to the action of a swelling agent which will modify the affinity of said portions for certain dyes, said treatment being of sufficient "severity" 40 to effect said change but less than that capable of producing any substantial swelling action on natural cotton fibres, and then dyeing the fabric to thereby produce different color tones in the treated and untreated portions.

7. The process of delusterizing the regenerated 50 cellulose fibre, which comprises subjecting the same to the action of an alkali of delustering strength and subsequently neutralizing the remaining alkali.

8. The process of ornamenting the regenerated cellulose, printing thereon with a paste in the desired pattern and subsequently subjecting said fabric to a bath, said paste or said bath including a caustic alkali.

55 9. A method for producing stiff fabrics that stand washing, which consists in manufacturing a mixed fabric composed of artificial silk fibres and of other fibres, and subjecting the mixed fabric to the action of an inorganic acid until the desired stiffening of the artificial silk is obtained, leaving the vegetable fibres soft and pliable.

10. The method for producing stiff fabrics that stand washing, which consists in manufacturing 65 a mixed fabric composed of artificial silk fibres and other fibres and subjecting the mixed fabric to the action of a cooled inorganic acid until the desired stiffening of the artificial silk is obtained, leaving the vegetable fibres soft and pliable.

70 11. A method for producing stiff fabrics that stand washing, which consists in manufacturing a mixed fabric composed of artificial silk fibres and of vegetable fibres, and subjecting the mixed 75

fabric to the action of an inorganic acid at atmospheric temperature until the desired stiffening of the artificial silk is obtained, leaving the vegetable fibres soft and pliable.

5 12. A stiff fabric that stands washing comprising a mixed fabric containing stiffened artificial silk and substantially unstiffened admixed threads.

10 13. The method of producing stiff, washable fabrics, which comprises manufacturing a mixed fabric containing artificial silk, and subjecting the fabric to the action of mineral acid, the concentration of the acid, the duration and temperature at which the fabric is subjected to said acid being such as to harden the artificial silk without materially affecting the other constituents of the fabric.

15 14. Artificial silk which has been subjected to the action of a swelling agent to structurally change the same and having at least one of its natural physical characteristics:—lustre, stiffness, translucency, thereby altered, the treatment being of sufficient severity to effect said

change but less than that capable of producing any substantial swelling action on natural cotton fibres.

15 15. Artificial silk which has been subjected to the action of a swelling agent to structurally change the same, having less lustre than the original silk and having at least one of its characteristics:—viz. stiffness, translucency, thereby altered, the treatment being of sufficient severity to effect said change but less than that capable of producing 10 any substantial swelling action on natural cotton fibres.

16. Artificial silk fabric with a pattern effect having localized portions which have been subjected to the action of a swelling agent to structurally change the same and having at least one of its natural physical characteristics:—lustre, stiffness, translucency, thereby altered, the treatment being of sufficient severity to effect said 15 change but less than that capable of producing 20 any substantial swelling action on natural cotton fibres.

GEORGES HEBERLEIN.

CERTIFICATE OF CORRECTION.

Patent No. 1,998,576.

April 23, 1935.

GEORGES HEBERLEIN.

It is hereby certified that error appears in the printed specification of the above numbered patent requiring correction as follows: Page 2, first column, line 29, after the word "with" insert the word the; page 3, first column, line 71, claim 1, for "treatment" read treatment; second column, line 62, claim 9, for "vegetable" read other; line 64, claim 10, for "The" read A; and line 67, for "other" read vegetable; and that the said Letters Patent should be read with these corrections therein that the same may conform to the record of the case in the Patent Office.

Signed and sealed this 25th day of June, A. D. 1935.

Bryan M. Battey

(Seal)

Acting Commissioner of Patents.